

## UNITED STATES PATENT OFFICE

2,158,652

## STEEL

Frederick M. Becket, New York, and Russell Franks, Niagara Falls, N. Y., assignors to Electro Metallurgical Company, a corporation of West Virginia

No Drawing. Application December 21, 1938,  
Serial No. 246,995

## 3 Claims. (Cl. 75—123)

This invention relates to steels, and provides new and improved steels characterized by novel and commercially valuable properties. This application contains subject-matter in common 5 with our application Serial No. 87,006, filed June 24, 1936.

We have discovered that the addition of columbium in amounts between 0.02% and 1% to so-called "plain carbon" and certain "low alloyed" steels effects a marked and surprising improvement in the properties of such steels. One important effect of the columbium addition is to refine the grain-size of the steel, and this grain refinement is retained and maintained 15 even at elevated temperatures up to and somewhat above the critical range. Another effect, which is doubtless at least in part a result of the grain refinement, is the improvement of the tensile strength of many of the steels. Further, 20 the impact strength is increased, and this improvement is marked even at subzero temperatures. There is also an increase in the resistance 25 of the steels to rusting and hot oxidation. The machinability and the deep-drawing and cold rolling characteristics of the steels are improved. The hardenability of the steels by heat treatment is somewhat decreased, and there is less distortion of the steel when it is rapidly cooled from elevated temperatures. The ratio 30 of yield point to maximum stress is increased, the increase depending upon the columbium and carbon contents of the steels: the increase is greater in the steels having the lower carbon and columbium contents.

35 Steels included in our invention are those containing up to 1% carbon, up to 1% silicon, up to 2% manganese, 0.05% to 5% nickel, 0.02% to 0.5% columbium, remainder iron.

Suitable amounts of columbium to be added to 40 these steels according to the present invention are from 0.02% to 0.5% columbium, and the most useful range is within the limits 0.05% to 0.25%. In general, the greater amounts of columbium should ordinarily be used in the steels containing 45 the greater amounts of carbon, within the ranges specified above.

One of the most valuable properties of the columbium containing steels of the invention is that of retaining its normally fine grained 50 structure at elevated temperatures, which property is attained without detrimentally affecting other important physical properties. The expedients heretofore customarily employed to refine the grain size of carbon and low-alloyed 55 steels have, in most cases, either detrimentally

affected the toughness of the steels, or failed to prevent coarsening of the grain size at elevated temperatures, during fabrication for instance, or both. The coarsening of the grain is considerably aggravated in a case carburizing process, and in such a process the addition of columbium to the steel is especially advantageous, as illustrated by the data in Table I which gives the experimentally determined grain number (A. S. T. M. Specification E 19-33) of the 10 cases of a series of steels after carburizing for eight hours at each of three different temperatures. In each case, the grain size of the core was smaller than that of the case.

Table I

| Composition of steel (remainder iron) |            |            |            |            | Grain No. of case after carburizing 8 hours— |            |              |
|---------------------------------------|------------|------------|------------|------------|----------------------------------------------|------------|--------------|
| Percent C                             | Percent Mn | Percent Si | Percent Cb | Percent Ni | At 925° C.                                   | At 975° C. | At 1,025° C. |
| 0.16                                  | 0.36       | 0.16       | None       | 3.49       | 2 to 6                                       | 2 to 6     | 2 to 7       |
| 0.37                                  | 0.40       | 0.17       | None       | 3.52       | 5 to 9                                       | 3 to 8     | 2 to 7       |
| 0.17                                  | 0.47       | 0.31       | 0.10       | 3.45       | 6 to 9                                       | 6 to 9     | 5 to 8       |
| 0.34                                  | 0.35       | 0.13       | 0.08       | 3.46       | 5 to 7                                       | 5 to 7     | 4 to 7       |
| 0.47                                  | 0.80       | 0.31       | 0.08       | 3.42       | 4 to 7                                       | 4 to 6     | 4 to 6       |

In general, the grain refining effect is roughly proportional to the columbium content up to a certain optimum amount of columbium, which optimum content depends chiefly on the carbon content of the steel. The grain refinement of a maximum 0.1% carbon steel reaches substantially its greatest degree at about 0.1% columbium; a 0.15% carbon steel at about 0.15% columbium; a 0.35% carbon steel at about 0.18% columbium; and a 0.5% carbon steel at about 0.25% columbium. A moderate excess of columbium above the optimum and below the maximum specified above (1%), will not ordinarily adversely affect the properties of the steel to a serious extent.

The influence of columbium on the tensile and impact properties of the steels under consideration is indicated by the data appearing in Table II which shows the experimentally determined yield point in thousands of pounds per square inch (Y. P.), maximum stress in thousands of pounds per square inch (M. S.), percentage 50 elongation in a 2 inch gage length (El. %), and reduction in area (R. A. %), all on 0.505 inch diameter A. S. T. M. standard tensile test pieces; and also the Izod impact value in foot pounds as determined on a standard Izod machine with 55

an initial energy level of 120 foot pounds and a standard specimen one centimeter square provided with a 45° notch.

Table II

| 5                                                       | Composition of steel<br>(remainder iron) |      |      |      |       | Tensile test |       |       |                |                  |
|---------------------------------------------------------|------------------------------------------|------|------|------|-------|--------------|-------|-------|----------------|------------------|
|                                                         | 10                                       | % C  | % Mn | % Si | % Ni  | % Cb         | Y. P. | M. S. | El.<br>Percent | R. A.<br>Percent |
| Quenched in oil from 900° C., drawn in air at 150° C.   |                                          |      |      |      |       |              |       |       |                |                  |
| 15                                                      | 0.16                                     | 0.36 | 0.16 | 3.49 | None  | 74           | 99.5  | 22    | 49             | 46               |
|                                                         | 0.17                                     | 0.47 | 0.31 | 3.45 | 0.10  | 63           | 102   | 21    | 39             | 57               |
|                                                         | 0.18                                     | 0.45 | 0.25 | 3.5  | 0.18  | 66           | 100   | 27    | 64             | 59               |
| Quenched in water from 875° C., drawn in air at 580° C. |                                          |      |      |      |       |              |       |       |                |                  |
| 20                                                      | 0.37                                     | 0.40 | 0.17 | 3.52 | None  | 116          | 120   | 7.5   | 21             | 23               |
|                                                         | 0.34                                     | 0.35 | 0.13 | 3.46 | 0.084 | 101          | 113   | 16    | 47             | 40               |
|                                                         | 0.32                                     | 0.45 | 0.25 | 3.5  | 0.13  | 97           | 115   | 22    | 60             | 41               |
| Quenched in oil from 850° C., drawn in air at 425° C.   |                                          |      |      |      |       |              |       |       |                |                  |
| 25                                                      | 0.51                                     | 0.76 | 0.25 | 3.5  | None  | 170          | 194   | 7     | 16             | 3.8              |
|                                                         | 0.47                                     | 0.80 | 0.31 | 3.42 | 0.084 | 175          | 191   | 12    | 37             | 8                |
|                                                         | 0.51                                     | 0.75 | 0.25 | 3.5  | 0.16  | 170          | 183   | 11    | 38             | 16               |
|                                                         | 0.54                                     | 0.75 | 0.25 | 3.5  | 0.46  | 170          | 184   | 12    | 41             | 11               |
| Air-cooled from 850° C.-900° C.                         |                                          |      |      |      |       |              |       |       |                |                  |
| 30                                                      | 0.16                                     | 0.36 | 0.16 | 3.49 | None  | 54           | 77    | 32    | 62             | 61               |
|                                                         | 0.17                                     | 0.47 | 0.31 | 3.48 | 0.10  | 70           | 82    | 27    | 50             | 73               |
|                                                         | 0.18                                     | 0.45 | 0.25 | 3.5  | 0.18  | 65           | 84    | 31    | 65             | 78               |
| 35                                                      | 0.37                                     | 0.40 | 0.17 | 3.52 | None  | 68           | 97    | 17    | 30             | 29               |
|                                                         | 0.34                                     | 0.35 | 0.13 | 3.48 | 0.084 | 72           | 94    | 25    | 43             | 37               |
|                                                         | 0.32                                     | 0.45 | 0.25 | 3.5  | 0.13  | 69           | 94    | 27    | 54             | 47               |
|                                                         | 0.51                                     | 0.76 | 0.25 | 3.5  | None  | 94           | 134   | 2     | 5              | 3.5              |
|                                                         | 0.47                                     | 0.80 | 0.31 | 3.42 | 0.084 | 102          | 144   | 10    | 15             | 5                |
|                                                         | 0.51                                     | 0.75 | 0.25 | 3.5  | 0.163 | 77           | 124   | 20    | 45             | 29               |
|                                                         | 0.54                                     | 0.75 | 0.25 | 3.5  | 0.462 | 82           | 131   | 17    | 56             | 19               |

40 As mentioned above, the addition of columbium to the plain carbon and low alloyed steels considerably increases their impact strength at sub-zero temperatures.

45 The presence of columbium substantially increases the resistance of these steels to hot oxidation and, although the columbium steels are not to be considered oxidation resistant in the sense that high chromium steels, for instance,

are oxidation resistant, the increase in resistance will be valuable in many uses of the steels.

The articles of the invention include articles deep-drawn from the steel of the invention; articles having a core containing less than 0.5% 5 carbon and a carburized case containing more than 0.8% carbon, and 0.02% to 0.5% columbium throughout; parts of machines and of other apparatus, required to withstand stress at moderately elevated temperatures; articles, composed of the steel of the invention, designed for use to resist impact shock at subzero temperatures; and pressure vessels, composed of the steel of the invention, designed to withstand two or three dimensional stress at subzero temperatures. 10

15 It will be appreciated that the specific examples herein are given by way of illustration, and that the invention is not limited to or by such examples.

We claim:

1. Steel containing carbon in an amount not exceeding 1%, manganese in an amount not exceeding 2%, silicon in an amount not exceeding 1%, 0.05% to 5% nickel, and 0.02% to 0.5% columbium, remainder iron; the columbium acting to impart to said steel a fine-grained structure which persists at all temperatures up to and somewhat above the critical range. 20

2. Steel containing carbon in an amount not exceeding 0.6%, manganese in an amount not over 2%, silicon in an amount not over 1%, 0.05% to 5% nickel, and 0.05% to 0.25% columbium, remainder iron; the columbium acting to impart to said steel a fine-grained structure which persists at all temperatures up to and somewhat above the critical range. 25

3. Case carburized article having a core containing less than 0.5% carbon and a carburized case containing more than 0.8% carbon, the core and case being composed of steel containing, aside from carbon, manganese in an amount not over 2%, silicon in an amount not exceeding 1%, 0.05% to 5% nickel, and 0.05% to 0.25% columbium, remainder iron; the columbium acting to impart to said carburized article a fine-grained structure, increased ductility, and increased impact strength. 40

FREDERICK M. BECKET.  
RUSSELL FRANKS.